

June 30, 1964

0, 1964 M. E. WEECH 3,139,4  
HIGH TEMPERATURE FURNACE FOR TREATING REFRACtORY MATERIALS  
WITH METALS AND INTERMETALLIC COMPOUNDS  
Filed Dec. 21, 1959

3,139,474

Filed Dec. 21, 1959



INVENTOR  
Marx E. Weech.  
BY Harness & Harris  
ATTORNEYS.

1

3,139,474

**HIGH TEMPERATURE FURNACE FOR TREATING REFRACATORY MATERIALS WITH METALS AND INTERMETALLIC COMPOUNDS**

Marx E. Weech, Idaho Falls, Idaho, assignor to Chrysler Corporation, Highland Park, Mich., a corporation of Delaware

Filed Dec. 21, 1959, Ser. No. 860,769  
17 Claims. (Cl. 13—31)

This invention relates to apparatus for and a method of treating base materials especially of refractory character with metals, intermetallic compounds or alloys of metallic elements. It especially concerns an electric resistance furnace in which said treatment may be practiced.

In my copending application Serial No. 747,497 filed July 9, 1958, I have described a method and apparatus whereby structures made of forms of allotropic carbon such as graphite, may be treated with a metal chloride vapor which will react with the carbon to form a metallic carbide layer or diffusion barrier that will protect the underlying carbon from corrosion and other attack by metals of high melting point character which may be handled or carried by the carbon structure. The present invention provides a furnace equipment and procedure for determining the diffusion resistance and barrier capabilities of the carbide coatings of refractory structures for instance of graphite treated in accordance with the invention of my copending application. Moreover, it provides a method for obtaining a metallic carbide interface on carbon base objects by treating the same with a molten metal which is to form the carbide, i.e. the vapor of said metal.

A feature of the invention is the provision of a high temperature electric resistance furnace having a current conducting, carbon resistance member shaped to provide a high resistance zone wherein heat treatment will be at its optimum.

Another object is to provide a high temperature resistance furnace employing a current conducting carbon resistance structure resiliently mounted between opposite current conducting members of opposite polarity.

A further object is to provide a high temperature resistance furnace as in the preceding object wherein the resilient mountings are provided by helical current conducting tubular coils which may also serve to conduct a cooling medium for cooling the region of contact between the current conducting members and the resistance structure.

An additional feature is the provision of a high temperature resistance furnace in which a plurality of shielding elements are provided surrounding the resistance element for cutting down heat losses in the heating zone.

Still another object is to provide a high temperature resistance furnace that includes a casing and cover wherein each is provided with fluid conducting heat exchange elements secured to each thereof.

A further object is to provide a method for treating an allotropic carbon structure with a high temperature metal forming a carbide of the metal at the interface between the metal and the carbon.

Still another object is to provide a method and high temperature furnace for checking the surface penetration of allotropic carbon receptacles having a metallic carbide facing, with a high temperature refractory metallic compound or alloy.

Other objects and advantages of my invention will be evident from the following description and from the drawing illustrating without restriction my invention as applied to a graphite crucible.

In the drawings:

FIGURE 1 is a schematic arrangement of a preferred

2

form of the apparatus of my invention, certain elements being shown in section and certain elements for purposes of clarity being shown of greater dimensional size than others;

5 FIGURE 2 is an enlarged view of a form of allotropic carbon structure to be treated and showing the manner of supporting the same; and

FIGURE 3 is a view partly in section of the liquid cooled cable.

10 In the drawing, similar numerals have reference to corresponding parts of the structure.

Referring especially to FIGURE 1, the numeral 10 generally refers to an electrical resistance furnace comprising a central current conducting and heating structure 15 preferably of graphite for instance a tubular current conducting resistance element 12, such as a cylindrical graphite pipe to which current is supplied at its opposite ends in any suitable manner preferably as hereinafter described. This element 12 preferably has a central longitudinal portion 14 between its ends 16, 18 formed, as by turning, with a wall 20 of reduced thickness to provide a preferred electrical resistance heating zone or path generally designated by the numeral 22 which is preferably of high resistance so as to provide a zone of high heat concentration. The element 12 is moreover preferably made of allotropic graphite having a density between about 1.6 to 1.9, the higher the density the greater the current and temperature produced for a given applied voltage.

30 The ends 16 and 18 of the resistance element 12 are preferably tapered to fit into contact with opposite current conducting resilient mounts in electrical connection with the source. These mounts comprise metallic conducting collars 24, 26 for instance of brass, which in turn nest in and are welded, silver soldered or brazed to the largest turn of the conically spirally wound spring coils 28, 30 which are constituted of tubular metal elements, the opposite ends of which extend through the cover 32 and casing 34 respectively of the metal housing 36, as shown, and are secured as by welding, silver soldering or brazing thereto in a manner to provide a rigid support for the coils and gas tight joint without effecting the resilience of the latter and to make good electrical connections. Thus the ends 38, 40 of the coil 28 extend through and are secured to the cover 32 and the ends 42, 44 of the coil 30 extend through and are secured to the wall 46 of the casing 34.

35 The coils 28 and 30 preferably have sufficient resilience to permit the current conducting structure such as the resistance element 12 to be releasably held between the collars 24, 26 with good electrical contact being maintained between these parts and between the collars 24, 26 and the coils 28, 30, which in turn have good electrical contact with the cover 32 and casing 36 respectively. It is a feature of the invention that the helical coils 28 and 45 20 serve as support or spring mountings and electrical conductors for the tubular element 12. They also serve to accommodate expansion and contraction of the element 12 and preferably act as liquid coolant conductors in heat exchange relationship with the collars 24, 26 for 50 cooling these collars and the end portions of the element 12 adjacent the zone 22 as hereinafter described.

55 The cover 32 is suitably secured as by cap screws 50 to a flange portion 52 of the casing 34. These cap screws 50 are suitably insulated as by plastic tubes 54, which may be of "Tygon" insulation, from the metal of the cover. A circular rubber O-ring seal 56 is provided between the cover 32 and flange 52 which is preferably provided with an O-ring groove 57 to provide a gas tight seal. Teflon rings 58 may be placed inside or outside 60 of the O-ring seal to minimize possibilities of short circuits between cover and casing.

Suitable electrical connectors generally designated by the numerals 59, 60 preferably made of heavy woven flexible copper cable 61 provided at their ends with solid copper terminals 62 and suitably liquid cooled as shown in FIGURE 2, are secured as by welding, silver soldering or bolting to extension straps or lugs 63 welded to the cover and casing respectively of the housing 36 and bring a high current of low voltage to the element 12.

As seen in FIGURE 3 showing one of the connectors, 59, 60, these are provided with flexible tubular sheaths 64 of synthetic plastic insulating material which are suitably cemented or sealed to shoulder portions 65 of the terminals 62. The sheaths are of a size to provide a space surrounding the cables 61 to which liquid coolant such as water may be circulated; suitable side tubular inlet and outlet connections 66 and 67 being provided for this purpose to be connected to a source of coolant and drain respectively. These connectors 59, 60 are in turn preferably connected to an A.C. single phase saturable reactor and isolation transformer (not shown) the high voltage side of which is connected to a source of power. Using a 2" internal diameter 14-inch long resistance tube 12, it is found possible to obtain temperatures up to about 4800° F. using the 9-volt output side of a 208 volt transformer at a current density of about 14 kw. By using a transformer with a 25-volt secondary, the temperature can be considerably higher up to 5500° and higher, the sole limitation being the vaporizing property of the carbon tube. In some cases due to the large current being conducted to the element 12, it may be desirable to provide separate flexible copper conductors 68, 69 between the collar 24 and the cover 32 and between the collar 26 and casing 34 respectively.

Arranged within the casing and suitably surrounding the resistance element 12 in spaced relation thereto is a radiation shield structure for reducing heat losses in the critical area 22. Such preferably comprises two or more inner tubular shields 70, 72 of a high melting point metal such as molybdenum or tantalum or other suitable refractory material of low emissivity (high reflectivity) arranged concentric with the element 12 and surrounded in turn by a single concentric stainless steel tubular radiation shield 74. These shields may be connected together by suitable tie bars 76 or wire preferably of molybdenum or tantalum and secured to the base of the housing 36 in any suitable manner as by screws (not shown) secured through foot extensions 80 of the radiation shields. The outer shield may alternatively rest in a groove cut in the base 46 and be positioned and supported radially by the groove.

In addition to the coils 28, 30 for cooling the ends of the element 12 there is preferably provided a plurality of independent copper coils in heat exchange relationship with the cover 32 and casing 34 of the housing and which are secured to the respective parts of the housing preferably by welding or silver soldering. FIGURE 1 shows a spirally wound copper tube section generally designated by the numeral 82 mounted on the cover 32 of the housing and which has an outer end or coil 84 connected through a plastic tube 86 with a source of liquid coolant such as water from a copper pipe line 88, 90, a suitable control valve 92 being located between the pipe sections 88 and 90 for controlling flow of the liquid coolant. The inner end of the section 82 is preferably connected to the end 38 of the copper coil 28 surrounding the upper end of the element 12, the opposite end 40 of this coil being connected by suitable plastic piping 93, and copper tubing 96, 98 with a drain 100. A funnel 102 is provided below the lower end of the copper tube sections 96 to give visual indication of the outflow of liquid coolant. Thus it will be seen that liquid coolant entering at 84 will flow through the coils of the section 82 leaving at the inner end thereof and entering the coil 28 at the inlet 38 and flowing through the coil

28 leaving at the outlet 40 thereof and entering the drain section 92. In certain cases it may be desirable to have the liquid coolant directly conducted from the input line 86 to the coil 28 inlet 38. In that event a branch line 104 is provided between the plastic section 86 and the inlet 38 and a discharge outlet section 106 is provided between the inner coil of the section 82 and discharge outlet pipe 40. Moreover, in order to inhibit deterioration of the sight glass gaskets 239, the cooling coil section 82 will preferably be extended up or down the sight glass tube 238 as at 83 in which case the free end of this extension will connect with the end 38 of the coil 28 or with the outlet 106 as the case may be.

A similar heat exchange section generally designated by the numeral 110 may be provided against the base wall 46 of the housing. This section has its outer coil inlet 112 connected by copper or synthetic plastic tubing 114, 116 with the pipe line 88 to bring liquid coolant to this section. The innermost coil has an outlet 118 which in turn connects by a copper or synthetic plastic tube conductor 120 with the pipe line 96 and thereby to the drain 100. An extension 122 of the inlet line 116 connects with the end 42 of the lower coil 30 supporting the element 12 to bring liquid coolant to such coil and the outlet extension 44 of the coil 30 is connected by a copper or synthetic plastic tubular section 124 with the discharge line 120 aforesaid. It will be understood that the section 110 and coil 30 may be interconnected as in the case of the upper coil 28 and section 82 to cause the liquid coolant to first traverse the section 110 and then the coil 30 and pass to the drain 100. A coolant fed heat exchange section is also provided surrounding the body 126 of the housing 36. This section preferably comprises two or more copper coil sections (three being shown) generally designated by the numerals 130, 132, and 134 each mounted as by welding or silver soldering to the body 126 of the housing for the purpose of cooling the body of the furnace when required which is desired prior to opening the furnace to remove a specimen. This cooling also prevents deterioration of the cover gasket. The uppermost section has its inlet 136 connected by a copper or synthetic plastic connector tube section 138 with the pipe line 88 of the source of liquid coolant and has its discharge end 140 connected by a copper or synthetic plastic section 142 with the discharge line 96 of the drain. Similarly, the inlet 144 of the section 132 is connected by a tube 146 with the liquid coolant feed line 88 and its discharge outlet 148 is connected by a connector tube 150 with the drain line 96. Similarly, the section 134 has its inlet 152 connected by a connector tube 154 with the liquid coolant feed line 88 and has its discharge outlet 156 connected by a connector tube 158 with the drain line 96. It will thus be apparent that each section of the housing as well as the current conducting end supports of the element 12 are provided with heat exchange devices for conducting heat away from the furnace.

The interior chamber 159 of the housing 36 is connected by a pipe line 160 with a series arranged vacuum pump 164 and a diffusion pump 166 through a shutoff valve 162, cold trap 163 and pipe 168. A suitable vacuum gauge 167, which may be of the "Phillips" ionization type is connected to the section 168 of the pipe line between the valve 162 and the diffusion pump 166 by a conductor 165 and is controlled by a valve 169. When the shutoff valve 162 is open it is possible to exhaust the air from within the chamber 159 and to operate the diffusion pump 166 for conveying the gases out of the furnace to establish a lower relative pressure than the vacuum pump 164 alone could attain. The pipe line 160 is also connected by a section 170 through a valve 172 with a source 174 of inert gas such as helium or argon. To indicate the pressure in the line 170 a manometer or pressure gauge 176 is provided which is connected by a pipe 178 through a valve 180 with the pipe section 170. Means for venting

the chamber 159 to atmosphere is provided by a valve 181 connected by a pipe 182 to the pipe line 161 between the chamber 159 and the valve 162.

Interiorly of the element 12 there is preferably provided a tubular metal base or coupling 200 secured as by welding to the base 46 of the housing and on which may be supported a graphite pedestal 202 having an end portion 203 of reduced section which fits within the metallic support 200. The upper end of the pedestal 202 preferably has a bore 206 forming a rim seat 208 for supporting an object or article to be treated with a high temperature boiling point metal. As seen in FIGURES 1 and 2, the object to be treated may for example be a graphite crucible 210 in which has been placed a quantity of a high boiling point metal 212 to effect such treatment. By preference a pedestal 202 of suitable length will be provided so as to position the crucible 210 and/or its contents preferably centrally, longitudinally of the wall 20, so as to place the same in the maximum temperature zone 22 provided thereby. The crucible in FIGURE 2 is shown to have a metal carbide surface strata 213 previously produced in accordance with the teachings of my copending application Serial No. 747,497 aforesaid. It will be understood that the treating metal 212 may be placed directly into a carbon crucible that does not have the previously formed metallic carbide surfacing.

The conditions prevailing in the furnace may be visibly determined as seen in FIGURE 1 by sighting an optical pyrometer generally designated by the numeral 234 through a clear viewing piece generally designated by the numeral 235 secured to the upper end of the furnace. The viewing piece may be an elongated tubular member 238 which may be an extension of the cover 32 or may be a separate tubular structure attached to the latter and of minimum size at the cover 32 and maximum size at the viewing end. The viewing piece 235 has a heat resisting clear window 236 suitably mounted and sealed therein by suitable heat resisting gaskets 239 as of synthetic rubber, between a flanged portion 240 of member 238 and a bezel 241 through bolts and nuts 242. As seen, the bezel 241 and flange portion 240 may be recessed as at 243, 244 to receive the window and gaskets, the lower one of which is preferably an O-ring. By means of the window visible observations of the temperature existing in the working area of the element 12 will be determinable.

In operation of the furnace 10, the article to be tested or treated, for example a crucible 210 made of carbon material such as graphite which is preferably pure and free of volatile materials such as hydrocarbons, is placed in the vacuum furnace as shown in FIGURE 1 and seated on the pedestal 202. This crucible may have previously been treated in accordance with the invention in my copending application aforesaid to obtain a suitable carbide layer, for example a titanium carbide surface layer 213 or strata within the hollow of the crucible, in which case the crucible is to be treated by placing a quantity of pure uranium within the crucible. If the crucible 210 is of an untreated character, its cup portion may for example be provided with a mixture of zirconium and bismuth for the purpose of obtaining a zirconium carbide layer at the interface.

Whatever the treatment to be accorded the article, the furnace 10 is then sealed so that it will hold a vacuum. Valve 92 is opened to permit flow of coolant water to the coils covering the casing and head of the furnace and to flow to the drain 100. Water also may be supplied to the cable sheathing inlets 66 to flow within the sheathing of the cables connecting the furnace terminals 63 with the transformer. The mechanical vacuum force pump 164 is then actuated and permitted to operate for several minutes or until the pressure at the inlet of the diffusion pump 166 reads between 100 to 500 microns of mercury absolute depending upon the type of diffusion pump employed or less if a McCleod or thermocouple gauge (not shown) on the same line as the ion gauge 167. Heat is

then turned on the boiler of the diffusion pump and the vacuum system allowed to pump the furnace down to an absolute pressure preferably in the range of 1-10 microns readable on the ion gauge 167. It is generally found that a lower pressure than one micron is not required and it is preferred to get down to 10 microns or less in order to remove most of the air from the furnace so that the air will not react with the material to be treated.

As soon as the system is pumped down to 1-10 microns, the power supply is connected to the local power distribution feeder, for example, a 208 volt, single phase system. About 30 volts of direct current is then applied to the saturable core reactor (not shown) in the power supply system, thus allowing current to flow through the reactor and through the isolation transformer (also not shown) which is in series with the reactor. The secondary of the isolation transformer is preferably connected through the water cooled large wires or cables 59 to the furnace at 63 so that large currents depending upon the characteristics of the transformer can be carried at voltages to be selected, for example 2500 amperes at a voltage of about 9 volts. The characteristics of the transformer will determine the temperature obtainable in the furnace within the capabilities of the current conducting.

The current is now allowed to flow from the cover 32 through coil 28, collar 24, tube 12, collar 26, coil 30 and casing 46 of the furnace at a relatively low rate until outgassing of the crucible, metal and furnace parts subside to low rates. The outgassing is usually substantially complete by the time the furnace has reached a temperature between 2000 to 2500° F. If the grades of graphite used aforesaid are such as to contain considerable volatile matter, it can take as long as an hour to heat a 30 or 40 gram graphite crucible of such material to a temperature of between 2000 to 2500° F. without exceeding a pressure of 25 to 50 microns at the diffusion pump inlet. On the other hand, if certain kinds of graphite, for example a spectroscopic electrode grade of low volatile content, is used a whole furnace top weighing about 400 grams can be subjected to full power in one step without releasing enough gas to raise the pressure at the diffusion pump by more than a few microns, for example, 5 to 10 microns for a few seconds, for example 30 seconds.

It is preferred to complete the outgassing step at low temperatures to minimize reaction of the gases with the metal to be heated. Once outgassing has been completed as evidence by a steady pressure of about 1 to 5 microns, power is applied to the furnace by decreasing the direct current voltage on the saturable reactor until the metal and article are heated to a temperature at which the metal 212 will melt and vaporize. This will occur when the vapor pressure of the melt exceeds the residual pressure in the chamber. At a voltage of 9 volts on the transformer secondary and a current flow of about 3000 amperes the temperature in the furnace at the zone 22, was about 4700 to 4800° F. At this temperature it was noted that the vapor pressure of the melt 212 exceeded the residual pressure in the chamber and there was some vaporization of the metal causing it to coat the inside of the resistance tube 12 with a carbide layer.

The furnace is allowed to run under desired power and predetermined temperature for about thirty minutes during which time the metal reacts with the hot object to produce a carbide interface if there has been no previous carbide layer on the inner surface of the crucible. Otherwise the metal should merely melt and/or vaporize. When the metal has been in molten condition for a sufficient length of time to carry out the desired coating at the interface or test on a previously coated crucible, the power is shut off and the power supply disconnected from the line. The furnace is then allowed to cool. Cooling may require from twenty to ninety minutes depending upon how vigorously cooling is supplied and how cool the treated part must be before withdrawal. After the furnace is cool, the valve 162 between the furnace and

the diffusion pump is shut, the vent valve 181 opened and air admitted to the furnace. The furnace is then unsealed by removing the top sight glass 236. The treated crucible 210 is then pulled out through the top sight opening.

The following examples will illustrate applications made of the furnace in connection with carbon crucibles.

*Example I*

A crucible previously provided with a smooth even and adherent coating of titanium carbide by the process of my copending application Serial No. 747,497 was placed in the furnace as shown in FIGURE 1. The furnace was first purged of air and other gases and a helium atmosphere admitted thereto at a pressure of 20 p.s.i. The crucible and coating were then subjected to repeated alternate cooling and heating cycles at temperatures of 700° F. to 2300° F. Cooling rates of 500° F. per minute were employed when lowering the temperature. The crucible and coating were subjected to 31 cycles of alternate heating and cooling after which the test was discontinued, there being no discernible change in the titanium carbide coating. This test established that thermal shock had no effect on the adherence of the titanium carbide coating to the carbon crucible and that it did not produce any change in the character of the coating.

*Example II*

A graphite crucible of the character of Example I having a titanium carbide coating on the interior face thereof was placed in the furnace conditioned with a helium atmosphere as described above in Example I after placing a quantity of uranium metal in the crucible. The crucible with its titanium carbide coating and uranium metal was heated to a temperature of 2300° F. and held at this temperature for four hours after which it was removed from the furnace. There was no evidence of any titanium carbide having been dissolved in the uranium. A number of tests of this character indicated that when the titanium carbide coating was thin some of the molten uranium penetrated the crucible wall to coat the exposed carbon and form uranium carbide therewith. Moreover that when the titanium carbide coating layer was of sufficient thickness it would serve as a complete barrier for preventing penetration of the molten uranium to the underlying graphite of the crucible.

*Example III*

A graphite crucible such as shown in FIGURE 1 and containing stoichiometric quantities of pure titanium sponge and carbon was placed in the furnace. The furnace was then purged of air and other gases and its temperature raised while being subjected to vacuum to a temperature of about 2900° F. sufficient to react the titanium and carbide to form titanium carbide. Test of the material indicated that it contained 99.7% pure titanium carbide.

*Example IV*

A three-gram sample of titanium carbide as prepared in Example III was placed in a crucible such as shown in FIGURE 1 containing uranium. The furnace was purged and then heated to 2400° F. and maintained at this temperature for four hours. During the heating, the uranium melted and the titanium carbide floated on the surface of the uranium. The furnace was thereafter cooled and a small fraction of the parent uranium removed for analysis. Analysis showed a maximum titanium content of 0.02%. This test demonstrated that the titanium carbide would not be broken down by heating in the presence of uranium.

From the foregoing description and examples, it will be evident that a novel furnace structure and method of treating refractory and other base materials with metals, intermetallic compounds and alloys of metallic elements has been disclosed according to which various resulting products may be obtained. It will be understood that numerous changes may be made in the details of con-

struction, in the process steps and in the ingredients employed without departing from the spirit and scope of the invention as set forth above and in the appended claims. For example, the processes described are not limited to the metals disclosed but may be applied to other refractory metals such as tungsten, tantalum or chromium.

I claim:

1. A furnace comprising a housing defining a gas tight chamber having opposite wall portions electrically insulated from each other, passage means connecting with said chamber through which a gaseous medium may be moved to or from said chamber, electric current conducting resistance heating means within said chamber having an interior chamber for receiving means to be acted upon by said furnace and having opposite generally tapering ends, a pair of coaxial mounts for said heating means within said chamber and free of fixed connection with said heating means, said mounts being arranged and constructed to provide a seating member axially adjacent each of said ends of said heating means having a face substantially complementary in shape to said tapering ends of said heating means and coil spring means acting axially of said heating means to resiliently and releasably clamp the said ends of said heating means between said faces in electrical contact therewith, one of said mounts being structurally connected with one of said wall portions and including means providing an electric current conducting path between said heating means and this one wall portion, and the other of said mounts being structurally connected with the other of said wall portions and including means providing an electric current conducting path between said heating means and said other wall portion.
2. A furnace as claimed in claim 1 wherein both of mounts includes said resilient supporting means for said heating means.
3. A furnace as claimed in claim 2 wherein each of said resilient supporting means is in the electric current conducting path between said heating means and said wall portions.
4. A furnace as claimed in claim 1 wherein said heating means is a tubular graphite element.
5. A furnace as claimed in claim 1 wherein said heating means is a tubular graphite element having a layer of metal carbide over its interior surface in the region of said element in which said means to be acted upon by said furnace is to be positioned.
6. A furnace as claimed in claim 1 wherein said heating means is a tubular graphite element and wherein there is a pedestal supported on one of said wall portions interiorly of said tubular element.
7. A furnace as claimed in claim 1 wherein each of said mounts comprises an annular collar having the said seating face and interengaged with said heating means, and a cooling coil interengaged with said collar.
8. A furnace as claimed in claim 7 where the means providing the electrical current conducting path between the heating means and the chamber wall portions comprises said collars and cooling coils of said mounts.
9. A furnace as claimed in claim 7 wherein the means providing the electrical current conducting path between the heating means and chamber wall portions comprises said collars and electrical conductors extending between said collar and wall portions around said cooling coils.
10. A furnace comprising a housing defining a gas tight chamber having opposite wall portions electrically insulated from each other, passage means connecting with said chamber through which a gaseous medium may be moved to or from said chamber, electric current conducting resistance heating means within said chamber having an interior chamber for receiving means to be acted upon by said furnace, a pair of supporting mounts for said heating means and between which said heating means is nested, each of said supporting mounts comprising a frustro conical support member for receiving an end portion of said heating means and a helical cooling coil mounted on and

in electrical contact with one of said wall portions and in electrical contact with and in a resilient supporting relation with said support member, and a pair of electrical conductor means for electrically connecting said wall portions of said housing with a source of electrical power for passing electric current through said wall portions, supporting mounts and heating means for heating the interior chamber of said heating means.

11. A furnace as claimed in claim 10 including at least one heat radiation shielding structure surrounding said heating means.

12. A furnace as claimed in claim 11 including means for establishing and maintaining a vacuum in said furnace.

13. A furnace as claimed in claim 10 wherein said electrical conductor means includes a fluid tight sheathing in non-electrical conducting relationship with said conductor means and providing a fluid containing space for receiving coolant fluid for cooling said conductor means.

14. A furnace comprising a housing defining a gas tight chamber having opposite wall portions electrically insulated from each other, passage means connecting with said chamber through which a gaseous medium may be moved to or from said chamber, electric current conducting resistance heating means within said chamber having an interior chamber for receiving means to be acted upon by said furnace, and a pair of mounts for said heating means and between which said heating means is nested, one of said mounts being structurally connected with one of said wall portions and providing an electric current conducting path between said heating means and this one wall portion, and the other of said mounts being structurally connected with the other of said wall portions and providing an electric current conducting path between said heating means and said other wall portion, each of said mounts including means providing a resilient support for said heating means relative to the wall portion with which such mount connects, said resilient supports being in the electric current conducting path between said heating means and the wall portion with which the mount connects and said resilient supports each comprising a cooling coil.

15. A furnace comprising a housing defining a gas tight chamber having two wall portions electrically insulated from each other, passage means connecting with said chamber through which a gaseous medium may be moved to or from said chamber, electric current conducting resistance heating means within said chamber having an interior chamber for receiving means to be acted upon by said furnace, a pair of generally coaxial electric current conducting support elements engaged with opposite ends of said heating means so to clamp said heating means between them, a cooling coil secured to and in electrical conducting relationship with one of said wall portions, said cooling coil also being an electrical conducting engagement and resilient supporting relationship with one of said pair of support elements, another cooling coil secured to and in electrical conducting relationship with the other of said two wall portions, said other cooling coil also

being in electrical conducting engagement and resilient supporting relationship with the other of said pair of support elements, and current conducting means connecting with said wall portions for conducting electrical current through said wall portions, cooling coils, and support elements to said heating means.

16. A furnace as claimed in claim 15 wherein each of said ends of said heating means has a straight tapered portion which interfits with a complementary tapered face on its associated support element, and wherein the cooling coils are helically wound to a conical shape and the support elements have outer tapered surfaces which interfit with a plurality of turns of the cooling coil.

17. A furnace comprising a housing defining a gas tight chamber having opposite wall portions electrically insulated from each other, passage means connecting with said chamber through which a gaseous medium may be moved to or from said chamber, electric current conducting tubular resistance heating means within said chamber providing an interior chamber for receiving means to be acted upon by said furnace, and a pair of mounts one at each end of said heating means and between which said heating means is releasably and resiliently clamped, one of said mounts being structurally connected with one of said wall portions and providing an electric current conducting path between said heating means and this one wall portion, and the other of said mounts being structurally connected with the other of said wall portions and providing an electric current conducting path between said heating means and said other wall portion, each of said mounts comprising a cooling coil and at least one of said cooling coils comprising resilient means providing a resilient connection for said heating means relative to the wall portion with which such mount connects.

35

#### References Cited in the file of this patent

#### UNITED STATES PATENTS

|           |                   |                |
|-----------|-------------------|----------------|
| 1,279,146 | Peacock           | Sept. 17, 1918 |
| 1,338,624 | Heppes et al.     | Apr. 27, 1920  |
| 1,513,890 | Bryan et al.      | Nov. 4, 1924   |
| 1,620,940 | Bleeker           | Mar. 15, 1927  |
| 1,700,942 | Lederer           | Feb. 5, 1929   |
| 1,858,062 | Ruckstahl         | May 10, 1932   |
| 1,981,015 | Williams          | Nov. 20, 1934  |
| 2,265,821 | Siegel            | Dec. 9, 1941   |
| 2,355,343 | Von Zeerleder     | Aug. 8, 1944   |
| 2,394,479 | Priessman         | Feb. 5, 1946   |
| 2,404,060 | Hall et al.       | July 16, 1946  |
| 2,756,166 | Alexander et al.  | July 24, 1956  |
| 2,768,277 | Buck et al.       | Oct. 23, 1956  |
| 2,778,866 | Sanz et al.       | Jan. 22, 1957  |
| 2,790,840 | Simmad et al.     | Apr. 30, 1957  |
| 2,798,108 | Poland            | July 2, 1957   |
| 2,969,448 | Alexander         | Jan. 24, 1961  |
| 2,971,039 | Westeren          | Feb. 7, 1961   |
| 3,009,974 | Sekkelsten et al. | Nov. 21, 1961  |